

# UNITED STATES PATENT OFFICE.

JAMES H. GRAVELL, OF ELKINS PARK, PENNSYLVANIA.

## METHOD OF AND COMPOSITION FOR CLEANING METALS.

1,387,645.

Specification of Letters Patent. Patented Aug. 16, 1921.

No Drawing.

Application filed February 27, 1920. Serial No. 361,699.

To all whom it may concern:

Be it known that I, JAMES H. GRAVELL, a citizen of the United States, residing at Elkins Park, in the county of Montgomery and State of Pennsylvania, have invented a certain new and useful Method of and Composition for Cleaning Metals, of which the following is a specification.

This invention relates to improvements in 10 metals and particularly to the cleaning of iron and steel, preparatory to painting.

The objects of the invention are, first, to provide a method and a composition or admixture for cleaning steel which will be 15 effective even when the metal is oily and rusty, and second, to provide an admixture operative by the action of an acid and adapted not only to remove excessive rust but also to remove grease, oil and the like, 20 and miscible with other ingredients and water whereby its action is hastened and its use simplified and facilitated.

In order to permit the acid of the compound or admixture to attack a rusty surface covered with a film of oil, I combine or admix with acid, benzol which a solvent of oils such as occur upon the surfaces of the metals to be cleaned and which is 25 peculiarly adapted for this purpose because it is miscible with other ingredients which I may use in my admixture and because in practice it has produced excellent results. An admixture of acid and benzol separates and although the admixture works satisfactorily in the hands of an expert workman, it cannot be used to advantage where care is 30 not exercised, so in order to overcome this difficulty, I add to the admixture a combining agent, such, for instance, as alcohol or acetone, which will dissolve or make 35 miscible both of the aforesaid ingredients, making a homogeneous fluid which does not require a skilful operator.

It will be understood by those skilled in 45 chemical operations that such an admixture would not rapidly act on a rusty surface, owing to the fact that little or no water is present to dissolve the resultant salts produced by the acid and I have discovered that 50 a certain amount of water may be added to the above admixtures without causing the ingredients to separate.

My admixture therefore primarily consists of an acid and benzol to which may 55 be added, to improve it, a liquid capable of dissolving the two or making them mis-

cible, and the admixture may still improve in its rapidity of action by the addition of water.

According to my invention the admixture 60 may be applied to the metal by brushing or spraying or the metal may be immersed in my admixture.

After the admixture has remained on the 65 surface of the metal a sufficient time to attack the surface, which may be both oily and rusty, the metal is washed with water and allowed to dry, in which case it is ready for further commercial operations such as 70 fabricating with dies or painting.

It is well known that such acids as sulfuric, nitric and hydrochloric cause the 75 steel to subsequently rust but I find that if a phosphoric or any other acid whose iron salts are permanent in the air is used, the steel is not only freed from this tendency 80 to rust but is practically put in a non-rusting condition, so that when phosphoric acid is used in my admixture, the admixture is highly valuable for preparing metal for 85 painting because metal treated according to my invention will not rust under the paint, even though it had a strong tendency to rust due to acid runs, hand-marks, soldering 90 solutions, etc., on the surface prior to the application of my admixture. I have found by experiment that the following formula produces a highly satisfactory cleaning 95 agent. The proportions given are by volume:

|                                |            |
|--------------------------------|------------|
| Phosphoric acid (85% solution) | .5 parts.  |
| Alcohol                        | 6.0 parts. |
| Benzol                         | 1.5 parts. |
| Water                          | .5 parts.  |

The proportions given in the above formula need not be exactly followed to produce satisfactory results as any proportions corresponding with the theory of my invention may be used.

As this invention is of a chemical nature it is evident to those skilled in the art that chemical equivalents may be substituted without departing from the spirit of the invention.

I claim:

1. The method of cleaning metal consisting in subjecting it to the action of an etching acid in the presence of benzol.
2. The method of cleaning metal consisting in subjecting it to the action of an admixture of an etching acid, benzol, and a

liquid with which said ingredients are miscible.

3. The method of cleaning metal consisting in subjecting it to the action of an admixture consisting of phosphoric acid and benzol.

4. The method of cleaning steel consisting in subjecting it to the solvent action of phosphoric acid, benzol, water, and a fluid in 10 which said ingredients are miscible.

5. A cleaning agent for metals consisting of an admixture of etching acid and benzene.

6. A cleaning agent iron and steel consisting of an etching acid, benzene, and a fluid in which said ingredients are miscible 15 to produce a homogeneous fluid.

7. A cleaning agent for metals consisting of an etching acid, benzene, water, and a fluid in which said ingredients are miscible to produce a homogeneous liquid. 20

8. A cleaning agent for iron and steel consisting of an admixture of phosphoric acid, alcohol, benzol and water.

JAMES H. GRAVELL.